

Dec. 21, 1937.

A. RUTTENAUER

2,103,093

GASEOUS ELECTRIC DISCHARGE LAMP DEVICE

Original Filed Dec. 2, 1936



INVENTOR  
Alfred Ruttenauer  
BY *Harry E. Dunham*  
ATTORNEY

## UNITED STATES PATENT OFFICE

2,103,093

GASEOUS ELECTRIC DISCHARGE LAMP  
DEVICEAlfred Ruttner, Berlin-Halensee, Germany,  
assignor to General Electric Company, a corpora-  
tion of New YorkApplication December 2, 1936, Serial No. 113,897.  
Renewed August 24, 1937. In Germany May  
30, 1936

10 Claims. (Cl. 176—122)

The present invention relates to gaseous electric discharge lamp devices having a gaseous filling comprising mercury vapor and a coating of luminescent material on the inner surface of 5 the lamp container.

It is frequently desirable to modify the appearance of the mercury vapor discharge in mercury vapor lamps and luminescent material, such as zinc silicate which emits a yellow light, 10 is useful for this purpose. It is possible to modify the typical blue-green appearance of the mercury vapor discharge tube by the addition of such yellow luminescent material to the extent that the tube has a white appearance. However, the mixed light of the mercury vapor discharge and the yellow luminescent material does 15 not contain all the colors found in daylight and for this reason this type of lamp device is more useful for outdoor advertising purposes 20 than for purposes of interior illumination.

The object of the present invention is to provide a mercury vapor discharge lamp having a coating of luminescent material on the inner surface thereof which lamp emits light similar 25 to daylight. Still further objects and advantages attaching to the device and to its use and operation will be apparent to those skilled in the art from the following particular description.

30 I have discovered that a mercury vapor discharge lamp having a coating of cadmium silicate on the inner surface of the lamp container emits light similar to daylight when the current density of the discharge is approximately 0.1-0.5 amp/cm<sup>2</sup> and when the cadmium silicate contains 0.5 to 0.1% manganese. These limits of current density and manganese content of the cadmium silicate are critical in obtaining light similar to daylight from a lamp 35 having the above structure. When the manganese content of the cadmium silicate is greater than 1% or less than 0.5% the light output of the material is not sufficient to balance the light output of the mercury vapor discharge so that the light emitted by the mercury vapor discharge preponderates in the light emitted by the lamp. When the current density of the discharge is greater than 0.5 amp/cm<sup>2</sup> the mercury vapor light preponderates in the 40 light emitted by the lamp and when the current density of the discharge is less than 0.1 amp/cm<sup>2</sup> the light emitted by the cadmium silicate preponderates in the light emitted by the lamp.

50 The light emitted by the cadmium silicate is

orange and thus has much more red in it than has daylight. This is desirable, however, since the luminescent light constitutes but a part of the total light output of the lamp and the excess of red in the luminescent light serves to 5 balance the light from the mercury vapor discharge which contains no red rays.

The light emitted by a lamp having the structure described above contains all the colors contained in daylight, that is the violet, blue, green 10 and yellow rays of the mercury vapor discharge and the yellow-red rays of the light emitted by the fluorescent material. While there is a slight color gap between the blue and the green mercury lines this is not of practical importance. 15

When light very closely approximating daylight is desired, for example in illuminating dyeing establishments, a luminescent material emitting a blue-green light is added to the cadmium silicate, which cadmium silicate is activated by 0.5 to 1% manganese. Preferably this luminescent material constitutes 10 to 30% of the cadmium silicate and is mixed therewith and applied to the inner surface of the lamp 20 container. Zinc tungstate or magnesium tungstate is preferred for this purpose. 25

In the drawing accompanying and forming part of this specification an embodiment of the invention is shown in a side elevational, partly 30 sectional view.

35 Referring to the drawing the gaseous electric discharge lamp device comprises an elongated tubular container 1 having electrodes 2 and 3 sealed therein at the ends thereof. The electrodes 2 and 3 are electron emitting when heated and consist of a pellet of electron emitting material, such as barium oxide, and a filament of high melting point material, such as tungsten, wrapped around said pellet. Said container 1 has a gaseous atmosphere therein consisting of a starting gas, such as argon, and a quantity 40 of vaporizable material, such as mercury, the vapor of which emits light during the operation of the device. A lamp having this structure is capable of operation with a discharge 45 current density of between 0.1-0.5 amp/cm<sup>2</sup>.

Said container 1 has a coating 4 of powdered luminescent material on the inner surface thereof (indicated by dotted lines in the drawing). The luminescent coating 4 consists of the material or materials disclosed above. The particles of luminescent material are applied to the inner surface of said container 1 by methods now known in the art, such as by first covering the inner surface of said container 1 with a volatilizable bind- 50 55

er, such as a mixture of glycerin and alcohol, and then applying the luminescent particles, as by dusting, to the binding material. The binder is then volatilized and removed from the container 5 1, as by heating and exhausting said container 1. A firmly adherent luminescent coating is thus applied to the inner surface of the container 1.

A lamp having the structure described above is an efficient light source useful for illuminating 10 purposes and the color of the light emitted thereby is similar to daylight.

It will be understood, of course, that I contemplate that numerous changes in the form and details of the device illustrated may be made by 15 those skilled in the art without departing from the spirit and scope of the invention, for example, the luminescent coating 4 may completely cover the inner surface of the container 1, or may be applied to selected portions of said surface, when 20 desired.

What I claim as new and desire to secure by Letters Patent of the United States is:—

1. A gaseous electric discharge lamp device comprising a container, electrodes sealed therein, 25 a gaseous atmosphere therein comprising mercury vapor and a coating of cadmium silicate associated with said lamp, said cadmium silicate containing from 0.5 to 1% manganese.

2. A gaseous electric discharge lamp device comprising a container, electrodes sealed therein, a gaseous atmosphere therein comprising mercury vapor and a coating of luminescent material associated with said lamp, said coating consisting of from 10 to 30% of fluorescent material emitting 30 green light and from 70 to 90% of cadmium silicate, said cadmium silicate containing from 0.5 to 1% manganese.

3. A gaseous electric discharge lamp device comprising a container, electrodes sealed therein, 40 a gaseous atmosphere therein comprising mercury vapor and a coating of luminescent material associated with said lamp, said coating consisting of from 10 to 30% of zinc tungstate and from 70 to 90% of cadmium silicate, said cadmium silicate 45 containing from 0.5 to 1% manganese.

4. A gaseous electric discharge lamp device comprising a container, electrodes sealed therein, a gaseous atmosphere therein comprising mercury vapor and a coating of luminescent material 50 associated with said lamp, said coating consisting of from 10 to 30% of magnesium tungstate and from 70 to 90% of cadmium silicate, said cadmium silicate containing from 0.5 to 1% manganese.

5. A gaseous electric discharge lamp device

comprising a container, electrodes sealed therein, a gaseous atmosphere therein comprising mercury vapor and a coating of cadmium silicate on the inner wall of said lamp and exposed to the discharge therein, said cadmium silicate containing from 0.5 to 1% manganese. 5

6. A gaseous electric discharge lamp device comprising a container, thermionic electrodes sealed therein, a gaseous atmosphere therein comprising mercury vapor and a coating of cadmium 10 silicate on the inner wall of said lamp and exposed to the discharge therein, said cadmium silicate containing from 0.5 to 1% manganese.

7. A gaseous electric discharge lamp device comprising a container, thermionic electrodes 15 sealed therein and supporting a discharge therein having a current density of the order of 0.1-0.5 amp/cm<sup>2</sup>, a gaseous atmosphere therein comprising mercury vapor and a coating of cadmium 20 silicate on the inner wall of said lamp and exposed to the discharge therein, said cadmium silicate containing from 0.5 to 1% manganese. 20

8. A gaseous electric discharge lamp device comprising a container, electrodes sealed therein, a gaseous atmosphere therein comprising mercury vapor and a coating of luminescent material on the inner wall of said lamp and exposed to the discharge therein, said coating consisting of from 10 to 30% of fluorescent material emitting 25 green light and from 70 to 90% of cadmium silicate, said cadmium silicate containing from 0.5 to 1% manganese. 30

9. A gaseous electric discharge lamp device comprising a container, thermionic electrodes sealed therein, a gaseous atmosphere therein comprising mercury vapor and a coating of luminescent material on the inner wall of said lamp and exposed to the discharge therein, said coating consisting of from 10 to 30% of fluorescent 35 material emitting green light and from 70 to 90% of cadmium silicate, said cadmium silicate containing from 0.5 to 1% manganese. 40

10. A gaseous electric discharge lamp device comprising a container, thermionic electrodes sealed therein and supporting a discharge therein 45 having a current density of the order of 0.1-0.5 amp/cm<sup>2</sup>, a gaseous atmosphere therein comprising mercury vapor and a coating of luminescent material on the inner wall of said lamp and exposed to the discharge therein, said coating consisting of from 10 to 30% of fluorescent material 50 emitting green light and from 70 to 90% of cadmium silicate, said cadmium silicate containing from 0.5 to 1% manganese.

ALFRED RUTTENAUER.

55